

June 20, 1967

A. C. SCURLOCK ET AL  
HIGH DENSITY METAL-CONTAINING PROPELLANTS  
CAPABLE OF MAXIMUM BOOST VELOCITY

Filed Oct. 28, 1960

3,326,732

7 Sheets-Sheet 1

Fig. 1.



INVENTORS

ARCH C. SCURLOCK,  
KEITH E. RUMBLE and  
MILLARD LEE RICE

BY

Martha L. Ross

AGENT

June 20, 1967

A. C. SCURLOCK ET AL  
HIGH DENSITY METAL-CONTAINING PROPELLANTS  
CAPABLE OF MAXIMUM BOOST VELOCITY

Filed Oct. 28, 1960

3,326,732

7 Sheets-Sheet 2



Fig. 2.

INVENTORS

ARCH C. SCURLOCK,  
KEITH E. RUMBLE and  
MILLARD LEE RICE

BY

Martha L. Ross

AGENT

June 20, 1967

A. C. SCURLOCK ET AL  
HIGH DENSITY METAL-CONTAINING PROPELLANTS  
CAPABLE OF MAXIMUM BOOST VELOCITY  
Filed Oct. 28, 1960

3,326,732

7 Sheets-Sheet 3

Fig. 3.



INVENTORS

Arch C. Scurlock,  
Keith E. Rumbel <sup>and</sup>  
Millard Lee Rice

BY

Martha L. Ross

AGENT

June 20, 1967

A. C. SCURLOCK ET AL  
HIGH DENSITY METAL-CONTAINING PROPELLANTS  
CAPABLE OF MAXIMUM BOOST VELOCITY

3,326,732

Filed Oct. 28, 1960

7 Sheets-Sheet 4

Fig. 4.



INVENTORS  
ARCH C. SCURLOCK,  
KEITH E. RUMBLE and  
MILLARD LEE RICE

BY

Martha L. Rose

AGENT

June 20, 1967

A. C. SCURLOCK ET AL  
HIGH DENSITY METAL-CONTAINING PROPELLANTS  
CAPABLE OF MAXIMUM BOOST VELOCITY

3,326,732

Filed Oct. 28, 1960

7 Sheets-Sheet 5

*Fig. 5.*



INVENTORS

ARCH C. SCURLOCK,  
KEITH E. RUMBLE and  
MILLARD LEE RICE

BY

*Martha L. Ross*

AGENT

June 20, 1967

A. C. SCURLOCK ET AL  
HIGH DENSITY METAL-CONTAINING PROPELLANTS  
CAPABLE OF MAXIMUM BOOST VELOCITY

3,326,732

Filed Oct. 28, 1960

7 Sheets-Sheet 6

*Fig. 6.*



INVENTORS

ARCH C. SCURLOCK,  
KEITH E. RUMBLE and  
MILLARD LEE RICE

BY

*Martha L. Ross*  
AGENT

June 20, 1967

A. C. SCURLOCK ET AL  
HIGH DENSITY METAL-CONTAINING PROPELLANTS  
CAPABLE OF MAXIMUM BOOST VELOCITY

3,326,732

Filed Oct. 28, 1960

7 Sheets-Sheet 7

Fig. 7.



INVENTORS  
Arch C. Scurlock  
Keith E. Rumbel and  
Millard Lee Rice

BY *Martha L. Ross*  
AGENT

## 1

3,326,732

## HIGH DENSITY METAL-CONTAINING PROPELLANTS CAPABLE OF MAXIMUM BOOST VELOCITY

Arch C. Scurlock, Arlington, Keith E. Rumbel, Falls Church, and Millard Lee Rice, Annandale, Va., assignors to Atlantic Research Corporation, Fairfax, Va., a corporation of Virginia

Filed Oct. 28, 1960, Ser. No. 65,860

20 Claims. (Cl. 149—19)

This invention relates to new propellant compositions. More specifically it relates to propellant compositions of high propulsive performance, which contain high density, metal fuel components.

The term propellant, as employed herein, refers to compositions comprising an organic fuel binder or matrix containing molecularly combined carbon and hydrogen, an oxidizer, and a finely-divided metal or metal hydride fuel. When introduced into the combustion chamber of a rocket motor and ignited such compositions generate high temperature gases, which vent out through the restricted nozzle of the motor at a high velocity to produce thrust.

The parameter generally accepted as indicative of the propulsive performance of a rocket propellant is its specific impulse, which is defined as the lbs. of thrust generated per lb. of propellant per second. Although this characteristic of the propellant is very important as a criterion for evaluating its performance, specific impulse is not the sole factor determining optimum performance in a specific application where the rocket system as a whole, including its inert parts, such as weight of the motor casing and payload, must be considered.

The usual objectives of rocket propulsion are the following:

- (1) Maximization of altitude and distance attained
- (2) Minimization of time-to-target
- (3) Maximization of thrust

Each of these objectives is accomplished by maximizing the boost velocity imparted to the rocket device by combustion of the propellant, the boost velocity being the velocity of the rocket at burn-out less velocity at launching.

We have found that the relationship between boost velocity and the characteristics of the propellant, obtained by applying Newton's second law of motion to the rocket, is defined, for an idealized rocket free of gravitational and drag effects and pressure thrust, by the following equation:

$$\Delta U = I_{sp} g_c \log \left[ 1 + \frac{\rho}{M_i/V_p} \right]$$

where

$\Delta U$ =boost velocity=velocity at burn out less launching velocity

$M_i$ =mass of inert parts including payload=mass of rocket less mass of propellant

$V_p$ =volume occupied of propellant

$I_{sp}$ =specific impulse of the propellant

$g_c$ =dimensional conversion factor,

32.17 (lb. mass) (ft.)/(lb. force) (sec.)<sup>2</sup>

$\rho$ =density of propellant

$M_i/V_p$ =mass-to-volume ratio

From this expression of the relationships which determine boost velocity, it will be seen that two additional factors, the density of the propellant and the ratio of the mass of inert parts to the volume of propellant enclosed within the motor, become exceedingly important, par-

## 2

ticularly at high  $M_i/V_p$  values, as in the case of boosters and JATO's. Under such conditions, a propellant having a lower specific impulse than that of another propellant can be more effective in terms of boost velocity if the density of the former is substantially higher. The specific impulse of the composition is, of course, an important factor since, obviously, as between two propellants of the same density, the one having the higher specific impulse will impart a higher boost velocity to a given rocket vehicle.

The effect of the specific impulse and density characteristics of the propellant and the  $M_i/V_p$  ratio is graphically shown in FIGURE 1, which compares the performance of a number of propellant compositions relative to a reference propellant, on propulsion of an idealized rocket vehicle, i.e. one for which the effects of drag, gravity, and pressure thrust are neglected, exhausting to 14.7 p.s.i. from a combustion chamber pressure of 1000 p.s.i. It will be noted that the effect of propellant density though substantial at relatively low  $M_i/V_p$  ratios, becomes increasingly important at such ratios increase. In the formulations shown, at high  $M_i/V_p$  ratios, the high density Zr propellant composition imparts a boost velocity which is as much as 27.5% higher than that imparted by the reference propellant, despite the lower specific impulse of the former. The low density oxygen-hydrazine propellant, on the other hand, despite its exceedingly high specific impulse, drops very considerably in propulsive performance at high  $M_i/V_p$  ratios.

From the foregoing discussion, it is evident that the boost velocity which is particular propellant can impart to the rocket vehicle in a specific application can be a more important practical yardstick than the specific impulse of the composition.

The object of this invention is to provide propellant compositions of high density, which are effective to impart maximized boost velocity to rocket vehicles or devices.

Other objects and advantages will become obvious from the following detailed descriptions and the drawings in which:

FIGURE 1 is a graph comparing the performance of several propellants of different specific impulse and density at different ratios of the mass of the inert parts of the rocket vehicle to volume of propellant.

FIGURES 2 through 7 are graphs comparing performance in terms of boost velocity and specific impulse of propellant formulations containing zirconium, zirconium hydride, thorium, uranium, and hafnium respectively.

Broadly speaking, the invention comprises propellant compositions consisting essentially of a finely divided solid, inorganic oxidizer and a finely-divided metal or metal hydride fuel selected from the group consisting of zirconium, uranium, hafnium, and thorium, and the hydrides of said metals, dispersed in an organic fuel matrix containing molecularly combined carbon and hydrogen, in which the oxidizer and fuel components are present in a particular ratio by weight in terms of the number of atomic equivalents, defined as follows:

$$\text{Oxidation Ratio} = \frac{O}{O + C + M \left( \frac{v}{2} \right)}$$

about 0.48-0.60, preferably 0.48-0.55

wherein O equals the total amount of oxygen in the propellant composition; C equals the total amount of carbon; M equals the total amount of metal calculated as free metal; and v equals the valence of the metal, preferably the characteristic valence of the metal in its most

stable oxide, which, in the case of Zr, Hf, Th and U, equals 4. Thus in the case of the following reaction:

$$\text{C} + \text{Zr} + 30 \rightarrow \text{CO} + \text{ZrO}_2$$

the Oxidation Ratio =  $\frac{3}{3 + 1 + 1\left(\frac{4}{2}\right)} = 0.5$

All molecularly combined oxygen, both in the inorganic oxidizer and in the organic fuel matrix, is included in the determination of total oxygen. Oxygen available for oxidation reaction, as, for example, the active oxygen present in the inorganic oxidizer or in an organic compound, such as a nitrate or nitrite derivative, functions to oxidize molecularly-combined carbon to CO and the metal fuel component to its oxide. Oxygen molecularly bonded to a carbon atom in an organic fuel compound, as, for example, in the case of an ether, alcohol, aldehyde, ketone, ester, amide, etc., though not available for combustion, nevertheless results, by decomposition reaction, in the formation of CO, the desired propulsive gas product. In cases such as organic acids, where decomposition might normally result in the production of CO<sub>2</sub>, under the conditions defined above for the Oxidation Ratio, one of the oxygen atoms preferentially combines with the metal fuel component.

When the components are present in a ratio by weight such that the Oxidation Ratio, as defined above, is 0.5, which will hereinafter be termed an OMOx formulation, the oxygen available for combustion of the fuel is stoichiometrically sufficient to oxidize the carbon not already linked to oxygen in the organic fuel to CO and the metal to its oxide. Under such conditions, the molecularly combined hydrogen in the organic fuel compound and in the metal hydride, if the latter is used, after ignition of the propellant composition, forms free hydrogen gas, since the molecularly combined carbon and the metal react preferentially with oxygen relative to the hydrogen. The hydrogen gas evolved is heated to a high temperature because of the high exotherm of the oxidizing metal. This, and its low molecular weight, make it a very efficient thrust-producing component in the combustion reaction product.

We have discovered that propellant formulations containing Zr, U, Hf, and Th, and their hydrides, as highly densifying, highly exothermic fuel components, impart the highest boost velocity to a rocket system of relatively high  $M_i/V_p$  ratio when the ratio of oxygen to fuel (organic and metal) is at OMOx or closely approaches OMOx, namely where the Oxidation Ratio equals about 0.48 to 0.60, the range 0.48 to 0.55 generally being preferred, although such formulations are not optimum with regard to specific impulse. These metal fuels, in such formulations, have the additional, highly advantageous characteristic of forming highly stable refractory oxides, which do not decompose or vaporize to any substantial degree after formation, either under the high temperature, high pressure conditions prevailing in the combustion chamber or during venting of the combustion gases out of the nozzle. Dissociation and/or vaporization of the metal oxides are undesirable since such phenomena absorb substantial amounts of heat energy, thereby reducing the temperature and pressure of the low molecular weight, thrust-producing combustion gases.

These findings are graphically illustrated by the data summarized on the curves in FIGURES 2 through 7. In all of these figures, boost velocity was determined at an  $M_i/V_p$  ratio of 60 lbs./cu. ft., assuming shifting chemical equilibria. In FIGURES 2 and 3, it will be seen that Zr at OMOx stoichiometry, both in a polyvinyl chloride fuel matrix plasticized with dibutyl sebacate and in a nitrocellulose-nitroglycerine, double-base matrix, with ammonium perchlorate as the solid oxidizer, gave the highest boost velocity, although, in both cases, these were not formulations having the highest specific impulse. FIG-

URES 4, 5, 6 and 7 show similar results for zirconium hydride, thorium, uranium, and hafnium.

The following comparative summary of the results obtained in double-base formulations, shows the effect of the density of the metal fuel component on boost velocity and the importance of the density factor relative to specific impulse at a high  $M_i/V_p$  ratio (60 lb./cu. ft.).

|                     | Metal Density | Metal Weight, Percent | OMOX     |       |
|---------------------|---------------|-----------------------|----------|-------|
|                     |               |                       | $I_{sp}$ | U     |
| Zr                  | 6.4           | 43.6                  | 229.2    | 9,180 |
| ZrH <sub>1.92</sub> | 5.5           | 44.0                  | 223.6    | 8,820 |
| Th                  | 11.4          | 57.2                  | 194.0    | 8,830 |
| Hf                  | 12.1          | 56.6                  | 198.0    | 9,130 |
| U                   | 18.9          | 63.2                  | 178.4    | 9,050 |

As aforementioned, the organic fuel matrix can be any suitable organic compound or mixture of organic compounds which contains molecularly combined carbon and hydrogen, so that at OMOx stoichiometry it burns and/or decomposes to produce CO and free hydrogen gas. It can be "inert", the term "inert" as used herein meaning a compound which requires an external source of oxygen, namely the solid, inorganic oxidier, for combustion. Illustrative of suitable organic matrix compositions are the various solid polymeric binders, such as polyether polysulfide, polyurethanes, butadiene-acrylic acid and -methacrylic acid copolymers cross-linked with an epoxy, alkyd polyesters, polyamides, cellulose esters, e.g. cellulose acetate, cellulose ethers, e.g. ethyl cellulose, polyvinyl chloride, asphalt, and the like. The oxygen linked to carbon in a variety of such inert fuel binders produces CO by decomposition reaction.

Many of the solid polymeric binders preferably include high-boiling, organic, liquid plasticizers to improve physical properties and processing of the propellant composition. Any of the numerous organic plasticizers known in the art and compatible with the propellant composition can be employed. Illustrative examples of suitable organic plasticizers include sebacates such as dibutyl sebacate and diethyl sebacate; phthalates, such as dibutyl phthalate and diethyl phthalate; adipates, such as diethyl adipate; glycol esters of higher fatty acids, and the like.

The organic fuel matrix can also comprise an active organic compound, a mixture of such compounds, or a mixture of such a compound with an inert organic compound, such as an inert organic plasticizer, the term "active" compound as employed herein meaning a compound which contains molecularly combined oxygen available for combustion of other components of the molecule, such as carbon. Examples of active organic fuel compounds include those containing nitroso, nitro, nitrite, and nitrate radicals, such as cellulose nitrate and nitroglycerine.

The foregoing description has dealt mainly with solid propellant compositions in which the organic fuel binder is a solid. The invention can also be employed in semi-solid, composite monopropellant systems. Such compositions are thixotropic, cohesive, shape-retentive compositions which can be extruded under moderate pressures into the combustion chamber of a rocket, where they form continuously advancing columns which burn on the exposed surface. In accordance with this invention, such plastic monopropellant compositions comprise a stable dispersion of a finely divided, insoluble oxidizer and the finely-divided heavy metal or heavy metal hydride in a continuous matrix of any suitable high-boiling organic liquid fuel containing molecularly combined carbon and hydrogen. Illustrative of suitable liquid fuels are hydrocarbons, such as triethyl benzene, liquid polyisobutylene, and the like; organic esters, such as dimethyl maleate, diethyl oxalate, dibutyl phthalate, and nitroglycerine; alcohols, such as benzyl alcohol and triethylene glycol; ethers, such as methyl  $\beta$ -naphthyl ether; and many others.

Any solid inorganic oxidizer can be employed which yields oxygen readily for combustion of the metal fuel component and the organic matrix, where the latter contains no oxygen or insufficient oxygen for CO stoichiometry. Such oxidizers include the inorganic oxidizer salts, such as NH<sub>4</sub>, K, Na, and Li perchlorates and nitrates, metal peroxides, such as CaO<sub>2</sub>, BaO<sub>2</sub>, and Na<sub>2</sub>O<sub>2</sub>, and the like, the salts being preferred.

Where the organic fuel matrix contains molecularly combined oxygen available in at least the stoichiometric amount required for oxidation and/or decomposition of the molecularly combined carbon component to CO, no inorganic oxidizer need be provided for its combustion. If such combined oxygen is present in amounts greater than that required for stoichiometry, the amount in excess preferentially oxidizes the powdered metal component rather than the molecularly combined hydrogen and thus can replace a portion of the inorganic oxidizer which would normally be required to oxidize the metal.

The organic fuel matrix, whether it be inert or active, solid or liquid, as aforescribed, must comprise at least about 20%, preferably at least 30%, by volume of the propellant composition. This is essential both to provide for generation of an adequate amount of low molecular weight combustion gases requisite for effective propulsion and for processing of a cohesive propellant composition having good physical properties.

The amounts of metal or metal hydride and solid, inorganic oxidizer employed must be such as to produce, with the particular organic matrix, an Oxidation Ratio within the specified range of about 0.48 to 0.60. This can readily be calculated by use of the equation given above for determination of this expression.

The following examples are illustrative of propellant formulations within the scope of the invention.

#### Example 1

The following components were thoroughly blended at room temperature:

|                                                              | Parts by weight |
|--------------------------------------------------------------|-----------------|
| Nitrocellulose (12.6% N) (spheres 10-12 microns in diameter) | 40 14.12        |
| Nitroglycerine                                               | 12.07           |
| Dibutyl phthalate                                            | 4.02            |
| Dibutyl sebacate                                             | 1.15            |
| Zirconium powder                                             | 45.90           |
| Ammonium perchlorate                                         | 22.10           |
| 2-nitrodiphenylamine                                         | 0.64            |

The slurry thus formed was heated to dissolve the nitrocellulose in the liquid mixture of nitroglycerine, dibutyl phthalate, and dibutyl sebacate to form a rigid gel containing uniformly dispersed therein the finely divided Zr and NH<sub>4</sub>ClO<sub>4</sub>. The Oxidation Ratio of the formulation is 0.59. Propellant grains made from this composition had a burning rate at 75° F. of 0.95 in./sec. at a combustion chamber pressure of 1200 p.s.i.

#### Example 2

The following components were thoroughly blended at room temperature:

|                                                                                                         | Parts by weight |
|---------------------------------------------------------------------------------------------------------|-----------------|
| Polyvinyl chloride                                                                                      | 6.46            |
| Diethyl adipate                                                                                         | 8.29            |
| Zr powder                                                                                               | 40.60           |
| Ammonium perchlorate                                                                                    | 44.40           |
| Wetting agent, equal parts glyceryl monooleate, pentaerythritol dioleate, diethyl sodium sulfosuccinate | 0.25            |

The slurry thus formed was heated to 350° F., at which temperature the PVC dissolved in the diethyl adipate to form a rigid gel matrix containing dispersed therein the Zr and NH<sub>4</sub>ClO<sub>4</sub>. The Oxidation Ratio of the formulation is OMOx. Burning rate of this composition at 75° F. was 0.5 in./sec. at 1000 p.s.i.

#### Example 3

A propellant composition was prepared as in Example 2 except that the components were in a somewhat different ratio by weight as follows:

|                    |       |
|--------------------|-------|
| 5 Binder:          |       |
| Polyvinyl chloride | 6.46  |
| Diethyl adipate    | 8.29  |
| Wetting agent      | 0.25  |
|                    | 15.00 |

|                                  |       |
|----------------------------------|-------|
| 10 Zr                            | 31.36 |
| NH <sub>4</sub> ClO <sub>4</sub> | 53.64 |

This composition is slightly oxygen-rich, the Oxidation Ratio being 0.578. Burning rate of the grain, static-fired in a motor, was 0.49 in./sec. at a motor chamber pressure of 950 p.s.i.

#### Example 4

20 A propellant composition was prepared as in Example 1 except that hafnium powder was substituted for Zr and the component proportions were varied. Ratio by weight of the binder was the same.

|                                                                                                      |      |
|------------------------------------------------------------------------------------------------------|------|
| 25 Binder: nitrocellulose, nitroglycerine, dibutyl phthalate, dibutyl sebacate, 2-nitrodiphenylamine | 30.0 |
| Hf                                                                                                   | 59.3 |
| NH <sub>4</sub> ClO <sub>4</sub>                                                                     | 10.7 |

30 This composition is OMOx. Burning rate at 1000 p.s.i. was 0.44 in./sec.

35 Although this invention has been described with reference to illustrative embodiments thereof, it will be apparent to those skilled in the art that the principles of this invention can be embodied in other forms but within the scope of the claims.

We claim:

1. In a rocket propellant composition which burns to produce propulsive gases and which consists essentially of a finely-divided, solid, inorganic oxidizer containing combined oxygen which it yields readily for combustion of the fuel components of said composition, and a finely-divided, solid metallic fuel component selected from the group consisting of Zr, U, Hf, Th and the hydrides of said metals, dispersed in an organic fuel matrix containing molecularly combined carbon and hydrogen, said organic fuel matrix comprising at least about 20 percent by volume of said composition, the improvement in which said oxidizer, said metallic fuel component and said organic fuel component are present in amounts such that the following expression:

$$\frac{O}{O+C+M\left(\frac{v}{2}\right)}$$

55 equals about 0.48 to 0.60 wherein O equals the total amount of combined oxygen in the composition; C equals the total amount of carbon; M equals the total amount of said metallic fuel component calculated as free metal, said O, C and M being expressed in terms of the number of atomic equivalents; and v equals the valence of said metal.

2. The propellant composition of claim 1 in which the organic fuel matrix comprises at least about 30% by volume of the composition.

3. The propellant composition of claim 2 in which the oxidizer is an inorganic oxidizer salt.

4. The propellant composition of claim 1 in which the metallic fuel component is Zr.

5. The propellant composition of claim 2 in which the metallic fuel component is Zr.

6. The propellant composition of claim 3 in which the metallic fuel component is Zr.

7. The propellant composition of claim 6 in which the organic fuel matrix comprises an organic polymer.

8. The propellant composition of claim 7 in which the organic polymer is plasticized with a high-boiling, organic liquid plasticizer.

9. The propellant composition of claim 8 in which the organic polymer is polyvinyl chloride.

10. The propellant composition of claim 6 in which the organic fuel matrix comprises nitrocellulose plasticized with nitroglycerine.

11. The propellant composition of claim 6 in which the oxidizer salt is ammonium perchlorate.

12. The propellant composition of claim 7 in which the oxidizer salt is ammonium perchlorate.

13. The propellant composition of claim 9 in which the oxidizer salt is ammonium perchlorate.

14. The propellant composition of claim 10 in which the oxidizer salt is ammonium perchlorate.

15. The propellant composition of claim 2 in which the expression:

$$\frac{O}{O+C+M\left(\frac{v}{2}\right)}$$

equals about 0.48 to 0.55.

16. The propellant composition of claim 1 in which  $v$  equals 4.

17. The propellant composition of claim 2 in which  $v$  equals 4.

18. The propellant composition of claim 5 in which  $v$  equals 4.

19. The propellant composition of claim 15 in which  $v$  equals 4.

20. The propellant composition of claim 19 in which the metallic fuel component is Zr.

#### References Cited

##### UNITED STATES PATENTS

2,931,437 4/1960 Smith ----- 52—0.5 X  
2,970,898 2/1961 Fox ----- 52—0.5

##### OTHER REFERENCES

Chem. and Eng. News, July 27, 1959, pp. 22, 23.  
Zaehringer, "Solid Propellant Rockets—Second Stage,"  
20 American Rocket Co., Box 1112, Wyandotte, Mich.  
(1958), pp. 214—216.

BENJAMIN R. PADGETT, Primary Examiner.

LEON D. ROSDOL, ROGER L. CAMPBELL, Examiners.